

1

3,671,292

## ZIRCONIUM ANTI-SOIL TREATMENT OF SYNTHETIC FIBERS AND RESULTANT ARTICLE

Julian J. Hirshfeld and Bertie J. Reuben, Decatur, Ala., assignors to Monsanto Company, St. Louis, Mo.  
No Drawing. Continuation-in-part of application Ser. No. 564,003, July 11, 1966, which is a continuation-in-part of applications Ser. No. 419,549, Dec. 18, 1964, and Ser. No. 419,601, Dec. 18, 1964. This application July 15, 1969, Ser. No. 841,977  
Int. Cl. D06m 11/04, 13/00

U.S. Cl. 117—62

17 Claims

### ABSTRACT OF THE DISCLOSURE

Durable anti-soiling characteristics are imparted to textile articles comprised of synthetic fibers by treating them with an acidic aqueous solution containing a zirconium salt and a derivative of ammonia, then drying the textile article thereby to bond the evaporation residue of the solution, a zirconium reaction product, to the synthetic fibers. The process may be varied by first treating the fibers with the zirconium salt followed by treatment with the derivative of ammonia.

This is a continuation-in-part application of co-pending application S.N. 564,003, filed July 11, 1966, entitled "Imparting Anti-Soiling Properties to Articles Comprised of Synthetic Fibers," which application, in turn, was a continuation-in-part application of co-pending application S.N. 419,549, filed Dec. 18, 1964, entitled "Process for Increasing the Resistance to Soiling of Polycarbamide Textile Articles" and S.N. 419,601, filed Dec. 18, 1964, entitled "Process for Increasing Resistance to Soiling of Acrylic Textile Articles," all now abandoned.

### BACKGROUND OF THE INVENTION

This invention relates to a process of treating textile articles to impart anti-soiling characteristics thereto and to textile articles treated by such a process. More specifically, the invention concerns a process of treating textile articles comprised of synthetic fibers with zirconium salts to impart anti-soiling characteristics thereto and to such articles treated by the process.

In the textile field and particularly in the carpet industry, where in recent years pastel colors and the use of carpets next to entrance ways have become popular, a need for anti-soiling characteristics built into textile articles has become more demanding. Also, the increased use of hydrophobic fibers, such as nylon, polyester, and acrylic, in textile articles has increased the need for anti-soiling properties since these fibers tend to accumulate static charges of electricity and, as a result, attract soiling particles.

Soiling of textile articles is generally effected by three methods, i.e., directly contacting the article with soiling particles, contacting the article with air-borne soiling particles, and contacting the article with liquid-borne substances containing soiling particles. Retention of these soiling particles on the textile article can be explained by three mechanisms, i.e., purely mechanical forces of entrapment or occlusion, interfacial adhesional forces such as Van der Wall's forces and electrostatic forces. Removal of the soiling particles from the textile article is dependent on

2

numerous factors. Generally speaking, large soiling particles can be readily removed whereas soiling particles within the range of less than 20 microns, and especially around 1 micron, are extremely difficult to remove from the textile article.

The textile industry has tried to prevent the soiling of textile articles by treating the articles with numerous organic and inorganic compositions. Most of these compositions are merely deposited on the article without any chemical bonding, and, as a result, are not effective over a prolonged period of time and are easily removed by washing, dry-cleaning or even vacuuming. For example, articles having interstices on the surface of the fiber are made soil-resistant by depositing small particles, usually less than 20 microns in diameter, of silicas on the fiber to fill the interstices and thus prevent the entrapment of soiling particles therein. However, most of these silicas do not chemically bond to the fiber and are easily removed by washing and vacuuming and, in some cases, cause dusting problems. Also, the textile industry has tried to prevent the build-up of static charges on hydrophobic fibers by treating these fibers with cationic softeners; however, limited success has been experienced since most of these softeners are usually water soluble and are readily removed by washing.

It is an object of this invention to provide a process for imparting anti-soiling characteristics to textile articles comprised of synthetic fibers.

Another object of this invention is to provide textile articles comprised of a synthetic fiber selected from the group consisting of polyamide fiber, polyester fiber, acrylic fiber, olefin fiber, modacrylic fiber, and spandex fiber with a process which imparts good anti-soiling characteristics thereto.

Other objects of the invention will become apparent as the invention is fully developed within the specification.

These and other objects of this invention are accomplished by providing a process of treating a textile article comprised of synthetic fibers comprising contacting the article with an acidic aqueous solution containing a zirconium salt and a nitrogen containing base, then drying the textile article, thereby to bond the evaporation residue of the solution, a zirconium reaction product, to the synthetic fibers.

The term textile article is meant to include fiber, yarn, all types of fabric, all types of carpets, and any textile article comprised of synthetic fiber. The term synthetic fiber is meant to include spandex fiber (a manufactured fiber in which the fiber-forming substance is any long-chain synthetic polymer composed of at least 85% by weight of a segmented polyurethane) polyester fiber (a manufactured fiber in which the fiber-forming substance is any long-chain synthetic polymer composed of at least 85% by weight of an ester of a dihydric alcohol and a dibasic acid or derivative thereof, such as terephthalic acid, or dimethylterephthalate), olefin fiber (a manufactured fiber in which the fiber-forming substance is any long-chain synthetic polymer composed of at least 85% by weight of ethylene, propylene, or other olefin units),

modacrylic (a manufactured fiber in which the fiber-forming substance is any long-chain synthetic polymer composed of less than 85% but at least 35% by weight of acrylonitrile units), nylon fiber (a manufactured fiber in which the fiber-forming substance is any long-chain synthetic polyamide having recurring amide groups

(—CO—NH—) as an integral part of the polymer chain), and acrylic fiber (a manufactured fiber in which the fiber-forming substance is any long-chain synthetic polymer composed of at least 85% by weight of acrylonitrile units). The textile article may contain minor amounts of material or fiber other than the synthetic fiber, e.g., jute backing in a carpet, etc.

The zirconium salts useful in the invention include any zirconium salt that is water soluble in the sense that they can be made soluble in water at certain pH's. Zirconium salts usually contain small amounts of hafnium, generally from about 0.5% to about 4.5% by weight. Hafnium is extremely similar to zirconium and, for purposes of this invention, it is to be assumed that where zirconium salts are mentioned herein it is meant to include zirconium salts with small concentrations, i.e., less than about 5.4% of hafnium. Examples of useful zirconium salts include zirconium acetate, zirconium oxychloride, zirconium sulfate, zirconium acetylacetone, potassium zirconyl carbonate, zirconium chloride, zirconium fluoride, zirconium nitrite, ammonium zirconyl carbonate, sodium zirconium oxychloride, sodium zirconium glycolate, and zirconium tetrachloride. From an economical standpoint, zirconium acetate is a particularly useful zirconium salt.

A nitrogen containing base is present in the acidic aqueous solution containing the zirconium salt. The nitrogen containing base can be either an organic or an inorganic derivative of ammonia. The organic nitrogen containing base can be a primary amine, a secondary amine, a tertiary amine, or a quaternary ammonium salt and can contain one or more groupings selected from the class consisting of alkyl, aryl, alkaryl and aralkyl. The groupings can contain substituents such as hydroxyl, carboxyl, sulfonic, nitro and halogens (chloro, bromo, fluoro, and iodo). Examples of useful inorganic nitrogen containing bases include hydroxylamine sulfate, hydroxylamine chloride, sulfamic acid, ammonium sulfamate, hydrazine, hydroxylamine, ammonia, and ammonium carbonate. Examples of useful organic nitrogen containing bases include ammonium carbamate, ethylene diamine, 1,6-hexamethylenediamine, guanidine, pyridine, monoethanolamine, glycine, aminoacetic acid, p-aminobenzoic acid, aniline, aniline hydrochloride, furfurylamine, o-toluidine, morpholine, N-methylfurfurylamine, N-methyltetrahydrofurfurylamine, and piperazine. The purpose of the nitrogen containing base is not completely explainable; however, it is known that the nitrogen containing base does help the deposition of the zirconium residue onto the fiber. In regards to fibers containing nitrogenous sites therein, it may be explained however, the explanation is not to be considered as a limitation hereof, that the nitrogen containing base forms a loose complex with the zirconium salt and this complex, due to its changed electrical characteristic, enables the zirconium salt to more readily attach itself to the nitrogenous sites in the fiber. More simply explained, the nitrogen containing base acts as a transfer agent or carrier for the zirconium compound. Its use results in a more durable deposition of the zirconium residue on the synthetic fibers than would otherwise be accomplished. The acidity of the aqueous solution should be within a pH range of from about 1.5 to less than about 7. Acids such as sulfuric acid, hydrochloric acid, acetic acid, phosphoric acid and formic acid are examples of acids useful to adjust the pH of the solution. Preferably, it is desired that the pH of the solution be within the range of from about 2 to about 5. The acidity of the aqueous solution helps to solubilize the zirconium salt and the nitrogen containing base, and to maintain the zirconium in solution until, when the article is dried, a zirconium residue is thereby uniformly deposited in the form of a microscopic cohesive and adhesive substantially continuous film of particles imbedded within the surface of the fibers. The zirconium salt should be present in the acidic aqueous solution in amounts ranging from about 0.2% to about 20.0%, and preferably within

the range of from about 1% to about 5%, the percents based on the weight of the textile article. Useful weight ratios of the zirconium salt to the nitrogen containing base within the acidic aqueous solution are from about 5:0.2 to about 1:1, and preferably about 5:3, respectively.

The temperature of the acidic aqueous solution should be within the range of from about room temperature to about 212° F. Higher temperatures, for example within the range of from about 175° F. to about the boiling point temperature of the solution are preferred in facilitating the contacting of the textile article with the acidic aqueous solution.

Contacting the textile article with the acidic aqueous solution can be accomplished by immersion, padding, spraying, exhaust bath, roll application and any other like means known in the textile art. The method of contacting should be adequate to completely wet the textile article with the solution. Contact time can vary from a few seconds to minutes or even hours. For example, where the acidic aqueous solution is padded on the textile article, the contact time can vary from about a half of a second to about 3 seconds; where an exhaust procedure is used, the contact time can vary from about 15 minutes to about 30 or more minutes; and where the article is immersed in the solution, the contact time can vary from about 5 minutes to about 90 minutes. Contact time should be measured from the time of contact of the solution described. If, for example, it should be desirable to introduce the nitrogen-containing base while the textile article is in contact with the acidic aqueous solution of the zirconium salt, contact time would be measured from the time of introduction of the nitrogen-containing base.

After the textile article is contacted with the acidic aqueous solution, the article is dried. Drying can be effected at temperatures within the range of from about room temperature up to about 350° F. Preferably, the textile articles are dried at temperatures within the range of 200° F. to 350° F.

Textile articles treated by the process of this invention exhibit good anti-soiling properties. Such properties are sufficiently affixed thereto to withstand dry-cleaning, washing, vacuuming, etc. Also, the textile article can be subjected to a dyeing process either before or after it is treated with the acidic aqueous solution of this invention.

The exact nature or explanation of why the textile articles treated by the process of this invention exhibit good anti-soiling properties is not fully understood. It is known that the zirconium residue is adequately bonded to withstand washing, dry-cleaning, and vacuuming.

The following examples are presented to illustrate the anti-soiling properties of the treated textile articles. All the samples used in the following examples are initially cleaned by scouring for 30 minutes at 160° F. in an aqueous solution (liquor to goods ratio being 40:1) containing 0.5% of a nonionic surfactant and 0.5% of tetrasodium pyrophosphate, percents based on weights of goods. After the samples are soiled, they are rinsed in cold water and dried at about 200° F. To show that the textile articles can be treated before being dyed, some of the samples are blank dyed. Such a blank dyeing procedure depends on the particular fiber. For example, where the fiber is a nylon fiber or an olefin fiber the sample is blank dyed by immersing it for 60 minutes in a boiling aqueous solution (liquor to goods ratio being about 35:1) containing about 0.5% (based on weight of goods) of a nonionic surfactant followed by rinsing and drying. Other blank dyeing procedures for particular fibers are of common knowledge in the art.

To illustrate the anti-soiling properties imparted to the textile articles, photo reflectance measurements or readings are made of two samples (dimensions being 2" x 4") of the textile article used in each example. Initial reflectance readings are made after the textile article is first treated in accordance with the invention and then

reflectance readings are made after the sample is soiled. The difference in the reflectance readings indicate the anti-soiling properties or characteristics of the samples, i.e. a large number indicates poor anti-soiling properties whereas a small number indicated good anti-soiling properties. The photo reflectance readings are measured by using a Photovolt Reflectance Meter (Model No. 610, Photovolt Corp., New York City, N. Y.). The samples of the textile articles are soiled by either of two methods, i.e. by an artificial soiling test or by a floor soiling test. The artificial soiling test is accomplished by placing the samples in a one gallon wide mouth jar having therein two glass rods (5 1/4" long by 3/8" diameter) glued on opposite sides of the jar and containing 10% (based on weight of the sample) of artificial soil and 10 number two rubber stoppers. The artificial soil has the following composition (the soil is sifted through a 30 mesh screen):

|                        | Percent |
|------------------------|---------|
| Peat                   | 22.3    |
| Silica gel             | 2.1     |
| Cement                 | 2.1     |
| Kaolin clay (peerless) | 2.1     |
| Molacco furnace black  | 0.2     |
| Red iron oxide         | 0.1     |
| Sawdust                | 52.5    |
| Calcium carbonate      | 10.9    |
| Animal charcoal        | 6.6     |
| Mineral oil            | 1.1     |
| Total                  | 100.0   |

The jar is then sealed, placed on a ball mill and rotated at 95-100 r.p.m. for 30 minutes in a clockwise direction and 30 minutes in a counter-clockwise direction at the same r.p.m. Thereafter, the samples are removed from the jar, vacuumized, and the photo reflectance readings of the two samples measured. The difference between the average initial reflectance readings and the average of the final reflectance readings indicate the degree of soil resistance. As mentioned earlier, a small photo reflectance difference number indicates a good anti-soiling property whereas a large number indicates a poor anti-soiling property of the textile article. The procedure in the floor soiling test is the same as the above artificial soiling test except the samples are soiled by placing them in the pathway of a well-traveled walkway and soiled by natural means, such as by shoes, air-borne soiling particles, etc. Control samples, that is samples that are not treated with the acidic aqueous solution containing the zirconium salt and the nitrogen containing base, are soiled under the same conditions as the test samples. The test results of the control samples as compared to the test results of the test samples indicate the significances of the invention. The percent increase in anti-soiling characteristic imparted to the samples is indicated in the examples as "Percent Improvement of Test Sample Over Control Sample." The initial reflectance readings of the control samples are taken after the control samples are scoured. Percents where used are based on weight unless otherwise specified.

#### Example 1

The following scoured samples are immersed in separate aqueous solutions (liquor to goods ratio 40:1) at room temperature, each solution has a pH of 2.4 and contains 1.1% zirconium acetate, 3% sulfuric acid and 3% hydroxylamine sulfate, the percents based on weight of the samples. The solutions are heated to and maintained at the boiling point for 30 minutes. Thereafter, the samples are removed from the solutions, rinsed in water, blank dyed, rinsed again in water, dried, and then subjected to the artificial soiling test. The results of the soiling test are indicated in Table I. Control samples, i.e. samples identical to their respective test samples except that they are not treated in the aqueous solutions, are presented to show the significance of the invention. 75

6  
TABLE I

|    |                                                                                                                                                                                                | Initial reflectance reading | Reflectance reading after soiling | Difference in reflectance readings | Percent improvement of test sample over control sample |
|----|------------------------------------------------------------------------------------------------------------------------------------------------------------------------------------------------|-----------------------------|-----------------------------------|------------------------------------|--------------------------------------------------------|
| 5  | (a) Nylon 6.6 knit (Cumuloft, a trademark of Chemstrand Company):                                                                                                                              |                             |                                   |                                    |                                                        |
| 10 | Control.....                                                                                                                                                                                   | 83                          | 27                                | 56                                 |                                                        |
|    | Test.....                                                                                                                                                                                      | 83                          | 39                                | 44                                 | 21                                                     |
| 15 | (b) Nylon 6.6 knit (601 Nylon, marketed by E. I. du Pont de Nemours & Company):                                                                                                                |                             |                                   |                                    |                                                        |
|    | Control.....                                                                                                                                                                                   | 80                          | 28                                | 52                                 |                                                        |
|    | Test.....                                                                                                                                                                                      | 80                          | 40                                | 40                                 | 23                                                     |
| 20 | (c) Nylon 6 knit:                                                                                                                                                                              |                             |                                   |                                    |                                                        |
|    | Control.....                                                                                                                                                                                   | 77                          | 24                                | 53                                 |                                                        |
|    | Test.....                                                                                                                                                                                      | 77                          | 33                                | 44                                 | 17                                                     |
| 25 | (d) Rayon knit:                                                                                                                                                                                |                             |                                   |                                    |                                                        |
|    | Control.....                                                                                                                                                                                   | 66                          | 25                                | 42                                 |                                                        |
|    | Test.....                                                                                                                                                                                      | 66                          | 30                                | 36                                 | 14                                                     |
| 30 | (e) Acrylic knit (copolymer containing 93% acrylonitrile and 7% vinyl acetate):                                                                                                                |                             |                                   |                                    |                                                        |
|    | Control.....                                                                                                                                                                                   | 67                          | 29                                | 38                                 |                                                        |
|    | Test.....                                                                                                                                                                                      | 68                          | 38                                | 30                                 | 21                                                     |
| 35 | (f) Acrylic yarn (Orlon type 33 Orlon a trademark of E. I. du Pont de Nemours & Co.):                                                                                                          |                             |                                   |                                    |                                                        |
|    | Control.....                                                                                                                                                                                   | 64                          | 33                                | 31                                 |                                                        |
|    | Test.....                                                                                                                                                                                      | 65                          | 37                                | 28                                 | 10                                                     |
| 40 | (g) Acrylic knit (90% acrylonitrile, 7% vinyl acetate and 3% vinyl bromide):                                                                                                                   |                             |                                   |                                    |                                                        |
|    | Control.....                                                                                                                                                                                   | 66                          | 30                                | 36                                 |                                                        |
|    | Test.....                                                                                                                                                                                      | 66                          | 40                                | 26                                 | 28                                                     |
| 45 | (h) Spandex knit (Blue "C," a trademark of Chemstrand Co.):                                                                                                                                    |                             |                                   |                                    |                                                        |
|    | Control.....                                                                                                                                                                                   | 71                          | 15                                | 56                                 |                                                        |
|    | Test.....                                                                                                                                                                                      | 72                          | 17                                | 55                                 | 1.8                                                    |
| 50 | (i) Polypropylene knit:                                                                                                                                                                        |                             |                                   |                                    |                                                        |
|    | Control.....                                                                                                                                                                                   | 75                          | 22                                | 53                                 |                                                        |
|    | Test.....                                                                                                                                                                                      | 77                          | 28                                | 49                                 | 7.5                                                    |
| 55 | (j) Acrylic yarn (76.5% being a copolymer of 93% acrylonitrile and 7% vinyl acetate, 10.5% being a copolymer of 50% acrylonitrile and 50% methylvinyl pyridine and 13% of polyvinyl chloride): |                             |                                   |                                    |                                                        |
|    | Control.....                                                                                                                                                                                   | 63                          | 38                                | 25                                 |                                                        |
|    | Test.....                                                                                                                                                                                      | 64                          | 51                                | 13                                 | 48                                                     |
| 60 | (k) Polyester knit (Blue "C," a trademark of Chemstrand Company):                                                                                                                              |                             |                                   |                                    |                                                        |
|    | Control.....                                                                                                                                                                                   | 82                          | 28                                | 54                                 |                                                        |
|    | Test.....                                                                                                                                                                                      | 83                          | 32                                | 51                                 | 6.6                                                    |

#### Example 2

Samples are treated as described in Example 1 except the solutions are at a pH of 3.7 and contain 3% acetic acid instead of the sulfuric acid. The results of the artificial soiling test are indicated in Table II.

TABLE II

|    |                                                                                 | Initial reflectance reading | Reflectance reading after soiling | Difference in reflectance readings | Percent improvement of test sample over control sample |
|----|---------------------------------------------------------------------------------|-----------------------------|-----------------------------------|------------------------------------|--------------------------------------------------------|
| 55 | (a) Nylon 6.6 knit (Cumuloft, a trademark of Chemstrand Company):               |                             |                                   |                                    |                                                        |
| 60 | Control.....                                                                    | 83                          | 27                                | 56                                 |                                                        |
|    | Test.....                                                                       | 83                          | 37                                | 46                                 | 18                                                     |
| 65 | (b) Nylon 6.6 knit (601 Nylon, marketed by E. I. du Pont de Nemours & Company): |                             |                                   |                                    |                                                        |
|    | Control.....                                                                    | 80                          | 28                                | 52                                 |                                                        |
|    | Test.....                                                                       | 81                          | 38                                | 43                                 | 17                                                     |
| 70 | (c) Nylon 6 knit:                                                               |                             |                                   |                                    |                                                        |
|    | Control.....                                                                    | 77                          | 24                                | 53                                 |                                                        |
|    | Test.....                                                                       | 78                          | 29                                | 49                                 | 7.5                                                    |
| 75 | (d) Rayon knit:                                                                 |                             |                                   |                                    |                                                        |
|    | Control.....                                                                    | 66                          | 24                                | 42                                 |                                                        |
|    | Test.....                                                                       | 66                          | 28                                | 38                                 | 9.5                                                    |
| 80 | (e) Acrylic knit (copolymer containing 93% acrylonitrile and 7% vinyl acetate): |                             |                                   |                                    |                                                        |
|    | Control.....                                                                    | 67                          | 29                                | 38                                 |                                                        |
|    | Test.....                                                                       | 65                          | 40                                | 25                                 | 34                                                     |

TABLE II—Continued

| Sample                                                                                 | Initial reflectance reading | Reflectance reading after soiling | Difference in reflectance readings | Percent improvement of test sample over control sample |
|----------------------------------------------------------------------------------------|-----------------------------|-----------------------------------|------------------------------------|--------------------------------------------------------|
| (f) Acrylic knit (90% acrylonitrile, 7% vinyl acetate and 3% vinyl bromide):           |                             |                                   |                                    | 5                                                      |
| Control                                                                                | 66                          | 30                                | 36                                 |                                                        |
| Test                                                                                   | 61                          | 36                                | 25                                 | 31                                                     |
| (g) Acrylic yarn (Orlon type 33, Orlon a trademark of E. I. du Pont de Nemours & Co.): |                             |                                   |                                    | 10                                                     |
| Control                                                                                | 64                          | 33                                | 31                                 |                                                        |
| Test                                                                                   | 64                          | 40                                | 24                                 | 23                                                     |
| (h) Spandex knit (Blue "C," a trademark of Chemstrand Company):                        |                             |                                   |                                    | 15                                                     |
| Control                                                                                | 71                          | 15                                | 56                                 |                                                        |
| Test                                                                                   | 72                          | 18                                | 54                                 | 3.6                                                    |

## Example 3

The following samples are treated as described in Example 1 except the aqueous solution is at a pH of 2.6 and contains 5% zirconium oxychloride, 3% hydrochloric acid and 3% hydroxylamine hydrochloride. The results of the soiling test are indicated in Table III.

TABLE III

| Sample                                                                                                                                                                                     | Initial reflectance reading | Reflectance reading after soiling | Difference in reflectance readings | Percent improvement of test sample over control sample |
|--------------------------------------------------------------------------------------------------------------------------------------------------------------------------------------------|-----------------------------|-----------------------------------|------------------------------------|--------------------------------------------------------|
| (a) Nylon 6.6 knit (Cumuloft, a trademark of Chemstrand Company):                                                                                                                          |                             |                                   |                                    | 40                                                     |
| Control                                                                                                                                                                                    | 83                          | 27                                | 56                                 |                                                        |
| Test                                                                                                                                                                                       | 83                          | 31                                | 52                                 | 7.1                                                    |
| (b) Nylon 6.6 knit (601 Nylon, marketed by E. I. du Pont de Nemours & Company):                                                                                                            |                             |                                   |                                    | 45                                                     |
| Control                                                                                                                                                                                    | 80                          | 28                                | 52                                 |                                                        |
| Test                                                                                                                                                                                       | 80                          | 31                                | 49                                 | 5.8                                                    |
| (c) Acrylic knit (copolymer containing 93% acrylonitrile and 7% vinyl acetate):                                                                                                            |                             |                                   |                                    | 50                                                     |
| Control                                                                                                                                                                                    | 67                          | 29                                | 38                                 |                                                        |
| Test                                                                                                                                                                                       | 67                          | 34                                | 33                                 | 13                                                     |
| (d) Acrylic yarn (76.5% being a copolymer of 98% acrylonitrile and 7% vinyl acetate, 10.5% being a copolymer of 50% acrylonitrile and 50% methylvinylpyridine and 13% polyvinyl chloride): |                             |                                   |                                    | 55                                                     |
| Control                                                                                                                                                                                    | 63                          | 38                                | 25                                 |                                                        |
| Test                                                                                                                                                                                       | 61                          | 51                                | 10                                 | 6                                                      |

## Example 4

Acrylic carpet samples composed of 76.5% of a copolymer being 93% acrylonitrile and 7% vinyl acetate, 10.5% of a copolymer being 50% acrylonitrile and 50% methylvinylpyridine and 13% polyvinylchloride are treated as described in Example 1 except that half of the samples are dyed a gold shade and half are blank dyed. The samples are subjected to the floor soiling test, results of the test are indicated in Table IV.

TABLE IV

| Sample               | Initial reflectance reading | Reflectance reading after soiling | Difference in reflectance readings | Percent improvement of test sample over control sample |
|----------------------|-----------------------------|-----------------------------------|------------------------------------|--------------------------------------------------------|
| (a) Dyed gold shade: |                             |                                   |                                    | 20                                                     |
| Control              | 31                          | 18                                | 13                                 |                                                        |
| Test                 | 31                          | 21                                | 10                                 | 23                                                     |
| (b) Blank dyed:      |                             |                                   |                                    | 25                                                     |
| Control              | 47                          | 25                                | 22                                 |                                                        |
| Test                 | 55                          | 38                                | 17                                 | 23                                                     |

## Example 5

Acrylic knit samples composed of 76.5% of a copolymer being 93% acrylonitrile and 7% vinyl acetate 10.5% of a copolymer being 50% acrylonitrile and 50% methylvinylpyridine and 13% polyvinylchloride are treated as described in Example 1 except the aqueous solution is at a pH of 3.9 and contains 3% ammonium sulfamate instead of the hydroxylamine sulfate. The results of the artificial soiling test are indicated in Table V.

TABLE V

| Sample      | Initial reflectance reading | Reflectance reading after soiling | Difference in reflectance readings | Percent improvement of test sample over control sample |
|-------------|-----------------------------|-----------------------------------|------------------------------------|--------------------------------------------------------|
| (a) Control | 53                          | 23                                | 30                                 |                                                        |
| Test        | 56                          | 30                                | 26                                 | 13                                                     |

## Example 6

Samples of acrylic knit are immersed for 30 minutes in boiling aqueous solutions (liquor to goods ratio being 30:1), the solutions containing compositions as outlined in Table VI. Thereafter the samples are removed from the baths, rinsed in water, blank dyed, rinsed again in water, dried and then subjected to the artificial soiling test. The results of the test are indicated in Table VI.

TABLE VI

| Sample      | Solution composition                                                        | pH of solution | Initial reflectance reading | Reflectance reading after soiling | Difference in reflectance readings | Percent improvement of test sample over control sample |
|-------------|-----------------------------------------------------------------------------|----------------|-----------------------------|-----------------------------------|------------------------------------|--------------------------------------------------------|
| (a) Control |                                                                             |                |                             |                                   |                                    |                                                        |
| (b) Test    | Zirconium acetate, 0.66%; hydroxylamine sulfate, 1.0%; sulfuric acid, 0.24% | 1.9            | 63                          | 51                                | 12                                 |                                                        |
| (c) Test    | Zirconium acetate, 1.1%; hydroxylamine sulfate, 3.0%; sulfuric acid, 0.4%   | 2.9            | 66                          | 60                                | 6                                  | 43                                                     |
| (d) Test    | Zirconium acetate, 1.1%; hydroxylamine sulfate, 1.0%; sulfuric acid, 0.4%   | 2.9            | 67                          | 57                                | 10                                 | 71                                                     |
|             |                                                                             |                |                             |                                   |                                    | 52                                                     |

9  
Example 7

Scoured samples of acrylic knit are treated as described in Example 1 except the aqueous solution contains 1.1% zirconium acetate (percent based on weight of sample), sulfuric acid to adjust the pH of the solution to the below indicated pH numbers, and 3% (percent based on weight of sample) of a nitrogen containing base as indicated in Table VII. Results of the artificial soiling test are indicated as difference in reflectance readings and are outlined in the following table, Table VII.

TABLE VII

| Sample      | Nitrogen containing base         | pH of solution | Difference in reflectance readings | Percent improvement of test sample over control sample |
|-------------|----------------------------------|----------------|------------------------------------|--------------------------------------------------------|
| (a) Control |                                  | 2.3            | -----                              | -----                                                  |
| (b) Test    | Hydroxylamine sulfate            | 2.9            | 13                                 | 44                                                     |
| (c) Test    | Hydrazine                        | 2.9            | 16                                 | 30                                                     |
| (d) Test    | Aniline                          | 2.4            | 12                                 | 48                                                     |
| (e) Test    | Aniline hydrochloride            | 2.1            | 15                                 | 35                                                     |
| (f) Test    | Furfurylamine                    | 2.3            | 15                                 | 35                                                     |
| (g) Test    | Ethylene diamine                 | 3.2            | 12                                 | 48                                                     |
| (h) Test    | 1,6-hexamethylene diamine        | 2.4            | 14                                 | 39                                                     |
| (i) Test    | o-Toluidine                      | 2.4            | 14                                 | 39                                                     |
| (j) Test    | Morpholine                       | 2.2            | 14                                 | 39                                                     |
| (k) Test    | N-methylfurfurylamine            | 2.2            | 13                                 | 44                                                     |
| (l) Test    | N-methyltetrahydro-furfurylamine | 2.2            | 13                                 | 44                                                     |
| (m) Test    | Piperazine                       | 2.3            | 16                                 | 30                                                     |
| (n) Test    | Hexamethylene tetramine          | 2.2            | 16                                 | 30                                                     |

## Example 8

Scoured samples of nylon knit are treated as described in Example 1 except the aqueous solutions (liquor to goods ratio being 30:1) contain compositions as outlined in Table VIII. The pH of the solutions and the results of the artificial soiling tests are indicated in the following Table VIII.

10  
TABLE IX

| Sample      | Nitrogen containing base         | pH of solution | Difference in reflectance readings | Percent improvement of test sample over control sample |
|-------------|----------------------------------|----------------|------------------------------------|--------------------------------------------------------|
| (a) Control |                                  | 6.0            | 44                                 | 6.4                                                    |
| (b) Test    | Ammonia                          | 3.6            | 32                                 | 32                                                     |
| (c) Test    | Hydrazine                        | 4.3            | 37                                 | 21                                                     |
| (d) Test    | Aniline                          | 3.5            | 38                                 | 19                                                     |
| (e) Test    | Aniline hydrochloride            | 4.7            | 29                                 | 38                                                     |
| (f) Test    | Furfurylamine                    | 3.7            | 34                                 | 28                                                     |
| (g) Test    | Ethylene diamine                 | 4.7            | 36                                 | 23                                                     |
| (h) Test    | 1,6-hexamethylene diamine        | 4.4            | 35                                 | 26                                                     |
| (i) Test    | o-Toluidine                      | 4.8            | 45                                 | 4.3                                                    |
| (j) Test    | Morpholine                       | 4.7            | 38                                 | 19                                                     |
| (k) Test    | N-methylfurfurylamine            | 4.7            | 38                                 | 19                                                     |
| (l) Test    | N-methyl tetrahydrofurfurylamine | 4.2            | 34                                 | 28                                                     |

The test samples treated as described in Examples 1-9 were subjected to repeated washing and vacuuming without deleteriously affecting their anti-soiling characteristics.

Although the above examples exemplify certain zirconium salts, nitrogen containing bases, textile articles and operating conditions, it is acknowledged and to be understood that equivalent zirconium salts, nitrogen containing bases, textile articles and operating conditions are also applicable and can be used with the invention.

What is claimed is:

1. A process for imparting semi-permanent anti-soiling characteristics to a textile article comprised of synthetic fibers comprising:

(1) Contacting the article with an acidic aqueous solution at a pH of from about 1.5 to less than about 7.0, at a temperature of from about room temperature to about the boiling point thereof, containing essentially as solutes from about 0.2% to about 20% of a water-soluble zirconium salt and from about 0.2% to about 20% of a material selected from the group consisting of organic and inorganic derivatives of ammonia, the percents based on the weight of the textile article; and

(2) then, drying the textile article thereby to bond the

TABLE VIII

| Sample      | Solution composition                                                          | pH of solution | Initial reflectance reading | Reflectance reading after soiling | Difference in reflectance reading | Percent improvement of test sample over control sample |
|-------------|-------------------------------------------------------------------------------|----------------|-----------------------------|-----------------------------------|-----------------------------------|--------------------------------------------------------|
| (a) Control |                                                                               | 77             | 33                          | 44                                | -----                             | -----                                                  |
| (b) Test    | Zirconium acetate, 0.44%; hydroxyl amine sulfate, 1.0%; and acetic acid, 3.0% | 4.1            | 77                          | 47                                | 30                                | 32                                                     |
| (c) Test    | Zirconium acetate, 1.1%; hydroxyl amine sulfate, 3.0%; and acetic acid, 3.0%  | 4.1            | 78                          | 59                                | 19                                | 57                                                     |
| (d) Test    | Zirconium acetate, 1.1%; hydroxyl amine sulfate, 1.0%; and acetic acid, 3.0%  | 4.1            | 77                          | 51                                | 26                                | 41                                                     |
| (e) Test    | Zirconium acetate, 1.1%; hydroxyl amine sulfate, 1.0%; and acetic acid, 3.0%  | 4.1            | 77                          | 50                                | 27                                | 39                                                     |
| (f) Test    | Zirconium acetate, 1.1%; hydroxyl amine sulfate, 1.0%; and acetic acid, 3.0%  | 4.1            | 77                          | 49                                | 28                                | 36                                                     |

## EXAMPLE 9

Scoured samples of nylon knit are treated as described in Example 1 except the aqueous solutions contain 1.1% of zirconium acetate (percent based on weight of goods), acetic acid to adjust the pH of the bath to the numbers indicated in Table IX and 3% (based on weight of the sample) of a nitrogen containing base as outlined in Table IX. The aqueous solution containing the ammonia does not contain acetic acid. Results of the artificial soiling test are indicated in Table IX.

evaporation residue of the solution, essentially a zirconium reaction product, to the synthetic fibers.

2. The process of claim 1 wherein the synthetic fiber is selected from the group consisting of polyamide fibers, polyester fibers, and acrylic fibers.

3. The process of claim 1 wherein the zirconium salt is zirconium acetate and the ammonium derivative is hydroxylamine sulfate.

4. The process of claim 1 wherein the acidic aqueous solution is at a temperature within the range of from

about 175° F. to about the boiling point temperature of the solution.

5. The process of claim 1 wherein the pH of the acidic aqueous solution is within the range of from about 2 to about 5.

6. The process of claim 1 wherein the acidic aqueous solution contains from about 0.4% to about 8.0% of the zirconium salt and from about 0.2% to about 5.0% of the ammonium derivative, the percents being based on the weight of the textile article.

7. The process of claim 6 wherein the zirconium salt is zirconium acetate and the ammonium derivative is hydroxylamine sulfate.

8. The process described in claim 1 wherein zirconium salt is selected from the group consisting of zirconium acetate, zirconium oxychloride, zirconium sulfate, zirconium acetylacetone, potassium zirconyl carbonate, zirconium chloride, zirconium fluoride, zirconium nitrite, ammonium zirconyl carbonate, sodium zirconyl oxychloride, sodium zirconium glycerinate, and zirconium tetrachloride; and said derivative of ammonia is selected from the group consisting of primary amines, secondary amines, tertiary amines, and quarternary ammonium salts.

9. The process of claim 8 wherein the synthetic fibers are selected from the group consisting of polyamide fibers, polyester fibers, and acrylic fibers.

10. The process of claim 8 wherein the acidic aqueous solution is at a temperature within the range of from about 175° F. to about the boiling point temperature of the solution.

11. The process of claim 8 wherein the pH of the acidic aqueous solution is within the range of from about 2 to about 5.

12. The process of claim 8 wherein the acidic aqueous solution contains from 0.4% to about 8.0% of the zirconium-containing material and from about 0.2% to about 5.0% of the ammonium derivative, the percents being based on the weight of the fibers.

13. A process for imparting semi-permanent anti-soiling characteristics to a textile article comprised of synthetic fibers comprising:

(1) Contacting the article with an acidic aqueous solution at a pH of from about 1.5 to less than about 7.0, at a temperature of from about room temperature to about the boiling point thereof, containing essentially as a solute from about 0.2% to about 20% of a water-soluble zirconium salt, the percentage based on the weight of the textile article;

(2) further contacting the article with from about 0.2% to about 20% of a material selected from the group consisting of organic and inorganic derivatives of ammonia, the percent being based on the weight of the textile article, and

(3) then drying the textile article thereby to bond the evaporation residue of the solution, essentially a zirconium reaction product, to the synthetic fibers.

14. A textile article comprised of synthetic fibers having bonded and embedded within the surface of said fibers, a microscopic uniform film of particles consisting essentially of the reaction product of a zirconium salt and a derivative of ammonia, said textile article having been produced by the process of (1) immersing the article in an acidic aqueous solution at a pH of from about 1.5 to less than about 7, at a temperature of from about room temperature to about the boiling point thereof, containing essentially as a solute about 0.2-20 percent of zirconium acetate and about 0.2-20 percent of a material selected from the group consisting of organic and inorganic derivatives of ammonia, the percents being based on the weight of the textile article; (2) then drying the article.

15. The textile article of claim 14 wherein the synthetic fiber is acrylic fiber.

16. The textile article of claim 14 wherein the synthetic fiber is a polyamide fiber.

17. A textile article comprised of synthetic fibers having bonded and embedded within the surface of said fibers a uniform microscopic uniform film of particles consisting essentially of a zirconium reaction product which is the residue of an evaporated acidic aqueous solution of from about 0.2% to about 20% of a water-soluble zirconium salt and from about 0.2% of a material selected from the group consisting of organic and inorganic derivatives of ammonia, the percents being based on the weight of the textile article.

#### References Cited

##### UNITED STATES PATENTS

|           |         |               |       |        |
|-----------|---------|---------------|-------|--------|
| 2,361,830 | 10/1944 | Edelstein     | ----- | 117-92 |
| 3,041,199 | 6/1962  | Miller et al. | ----- | 117-62 |
| 3,058,850 | 10/1962 | Sell          | ----- | 117-76 |
| 3,450,555 | 6/1969  | Bridgeford    | ----- | 117-62 |
| 3,429,647 | 2/1969  | Yao et al.    | ----- | 8-21   |

##### OTHER REFERENCES

Blumenthal: Zirconium Chemicals Their Application to Textiles, Rayon and Synthetic Textiles, pp. 81-83, December 1950.

WILLIAM D. MARTIN, Primary Examiner

R. HUSACK, Assistant Examiner

##### U.S. CL. X.R.

117-138.8 N, F, VA, E, D, 139.5 CQ, CF, 169; 252-8.6